# EUROPEAN PATENT SPECIFICATION

(11) **EP 1 623 839 B1**
(45) Date of publication and mention of the grant of the patent: **25.06.2008**
(21) Application number: 05016941.6
(22) Date of filing: 04.08.2005
(51) Int. Cl.: B41M 1/28, B44C 3/00

(54) **Method for making metallized and metallized-pigmented transfer printings and the transfer printing obtainable thereby**
Verfahren zum Erzeugen von metallisierten und metallisiert-pigmentierten Transferdrucken und Drucke welche dadurch herstellbar sind
Procédé pour réaliser par transfert des impressions métallisées ainsi que métallisées pigmentées et impressions ainsi réalisables

(30) Priority: 05.08.2004 IT MI20041616
(43) Date of publication of application: 08.02.2006
(73) Proprietor: Transfer Gomma S.r.l., 35030 Saccolongo PD (IT)
(72) Inventor: Aldinio Colbachini, Paolo, 36040 Montegalda (Vicenza) (IT)
(74) Representative: Cicogna, Franco

(56) References cited:
- US-A- 4 398 994
- US-A- 4 781 792
- US-A- 4 915 780

## Description

### BACKGROUND OF THE INVENTION

The present invention relates to a method for making metalized and metalized-pigmented transfer printings.

The invention also relates to the transfer printing made by the above method.

The field of the invention is that of the methods for making metalized transfer printings, i.e. support elements (usually made of a sheet clear plastics material) supporting wordings, patterns, figures or the like thereon, made by starting from a metal film, in particular an aluminium film, and which are transferred, by pressure and heating, on a surface to be patterned.

Prior transfer printings have been made by removing, by acid solutions, the metal material, to form the target or desired pattern.

However, the use of acid solutions is affected by great drawbacks, related to the liquid phase of the reactive material (which can be hardly controlled in the desired processing operations), and the acid nature of the medium, requiring difficult and complex operations in the printing process, which greatly increase the total processing time.

Moreover, the above mentioned prior transfer printings do not provide a quality and resolution image.

US 4 915 780 relates to a process for making metallized sheets for microwave heating having varying densities of metal at different locations thereon, in order to provide different degrees of heating in different regions of the metallized sheet upon the application of microwave energy.

### SUMMARY OF THE INVENTION

Accordingly, the main object of the present invention is to provide a novel method for making metal transfer printings which, with respect to the above mentioned prior methods, which is much more simple, quick and, moreover provides high quality and resolution images.

A further object of the present invention is to provide such a method which also allows to make metalized-pigmented transfer printings, i.e. transfer printings the images or patterns of which are made by a pigmented composition on a metal material.

According to one aspect of the present invention, the above mentioned aim and objects, as well as yet other objects, which will become more apparent hereinafter, are achieved by a method and transfer printings as claimed respectively in claims 1 and 4.

Further preferred embodiments of the invention are pointed out in the other claims.

With respect to prior screen printing method, the inventive method provides the advantage that it allows to make transfer printings in a much more simple and quick manner, thereby allowing to obtain high quality and resolution image, having a image definition or resolution greatly improved with respect to the image which can be obtained by prior transfer printings.

### BRIEF DESCRIPTION OF THE DRAWINGS

Further characteristics and advantages of the invention will become more apparent hereinafter from the following detailed disclosure of a preferred embodiment of the invention which is illustrated, by way of an indicative, but not limitative, example in the figures of the accompanying drawings.

In the drawings:
Figure 1 shows a block diagram of the method according to the present invention; and
Figures 2 and 5 show the operating steps of the method shown in figure 1.

### DESCRIPTION OF THE PREFERRED EMBODIMENT

With reference to the above mentioned figures, the method according to the present invention comprises a starting coupling operating step, in which, by using a glue layer 3, a metal material film 1, either colored or not, is coupled or applied on a supporting sheet element 2, made of a plastics material, either clear or neutral, preferably a polyester resin.

Then by a screen printing operation, a plastic resin is printed on the film 1, thereby coating the area 4 of the image of pattern to be reproduced on the transfer printing element.

To remove from the film 1 the uncovered metal surface, i.e. the surface on the outside of the image pattern 4, said film is processed in a delaminating step, which is carried out by spreading on the overall surface of the film a basic mixture or paste, thereby providing a layer 5 adhering to and covering both the image or pattern 4 and the remaining surface of the film 1.

Preferably, the mixture or paste forming said layer 5 is based on sodium hydroxide, as added with an inert filler.

Then, by suitable washing or sensing steps, from the supporting sheet element 2 is removed the film portio1 1 left uncovered by the screen printing resin, while holding unaltered the protected part or surface of the film 4 corresponding to the transfer image or pattern.

After a following drying step, a transfer printing is obtained which can be subjected to any desired screen printing operations, to provide the image or pattern with the desired colors.

Advantageously, the used film 1 can be of any desired metal types, in particular, aluminium or pigmented aluminium.

In the latter case, the delaminating step is carried out by adding to the basic mixture or paste, for forming the above mentioned layer 5, with suitable organic solvents, adapted to remove the pigmentation on the unprotected areas or regions of the film 1.

## Claims

1. A method for patterning a surface comprising the steps of:
(a) forming a metalized base or metalized-pigmented base printable film by coupling, through a glue layer, a metal film onto a supporting sheet element;
(b) screen printing, on said printable film, an image or pattern by using a protective resin coating;
(c) delaminating the portion of the film which is not coated by said protective resin by spreading, on the overall surface of the film, a basic mixture or paste containing inert filler materials;
(d) removing by washing said film delaminated portion;
(e) drying the metallized printing, and
(f) transferring, by pressure and heating, the thus obtained on the surface to be patterned.

2. The method according to claim 1, **characterized in that** said method further comprises additional screen printing steps for coloring the printed image or pattern.

3. The method according to claim 2, **characterized in that** said basic mixture comprises organic solvents for the pigments.

4. The method according to claim 3, **characterized in that** said method further comprises the step of carrying out additional washings of unprotected areas, by using organic solvents adapted to remove said pigments.

5. The method according to claim 1, **characterized in that** said basic mixture or paste is a sodium hydroxide and inert filler material mixture or paste.

6. A metalized or metalized-pigmented transfer printing, **characterized in that** said printing is made by a method according to one or more of the preceding claims.

## Patentansprüche

1. Verfahren zum Strukturieren einer Oberfläche, folgende Schritte umfassend:
(a) Bilden einer bedruckbaren Folie auf metallisierter Basis oder metallisiert-pigmentierter Basis durch Verbinden einer Metallfolie mit einem tragenden Bahnelement mittels eine Klebstoffschicht,
(b) Siebdrucken eines Bildes oder einer Struktur auf die bedruckbare Folie unter Verwendung einer schützenden Harzbeschichtung,
(c) Ablösen des Abschnitts der Folie, die nicht mit dem schützenden Harz beschichtet ist, durch Aufbringen einer Basismischung oder -paste, die inerte Füllmaterialien enthält, auf die gesamte Oberfläche der Folie,
(d) Entfernen des abgelösten Abschnitts des Filmes durch Waschen,
(e) Trocknen des metallisierten Drucks und
(f) Übertragen des so Erhaltenen auf die zu strukturierende Oberfläche durch Druck und Erhitzen.

2. Verfahren nach Anspruch 1, **dadurch gekennzeichnet, dass** das Verfahren ferner zusätzliche Siebdruckschritte zum Färben des gedruckten Bildes oder der Struktur umfasst.

3. Verfahren nach Anspruch 2, **dadurch gekennzeichnet, dass** die Basismischung organische Lösemittel für die Pigmente umfasst.

4. Verfahren nach Anspruch 3, **dadurch gekennzeichnet, dass** das Verfahren ferner den Schritt des Ausführens weiterer Waschungen der ungeschützten Bereiche unter Verwendung organischer Lösemittel umfasst, die dafür angepasst sind, die Pigmente zu entfernen.

5. Verfahren nach Anspruch 1, **dadurch gekennzeichnet, dass** die Basismischung oder -paste eine Mischung oder Paste aus einem Natriumhydroxid und einem inerten Füllmaterial ist.

6. Metallisierter oder metallisiert-pigmentierter Transferdruck, **dadurch gekennzeichnet, dass** der Druck mit einem Verfahren nach einem oder mehreren der vorhergehenden Ansprüche ausgeführt wird.

## Revendications

1. Procédé permettant de former un motif sur une surface comprenant les étapes suivantes:
(a) formation d'un film imprimable à base métallisée-pigmentée ou à base métallisée en couplant, par le biais d'une couche de colle, un film métallique à un élément de feuille de support;
(b) impression en sérigraphie, sur ledit film imprimable, d'une image ou d'un motif en utilisant un revêtement de résine protectrice ;
(c) délaminage de la partie du film qui n'est pas revêtue de ladite résine protectrice en étalant, sur toute la surface du film, une pâte ou un mélange de base contenant des matériaux de charge inerte ;
(d) retrait, par lavage, de ladite partie délaminée du film ;
(e) séchage de l'impression métallisée, et
(f) transfert, par pression et chauffage, du résultat ainsi obtenu sur la surface sur laquelle doit être formé le motif.

2. Procédé selon la revendication 1, **caractérisé en ce que** ledit procédé comprend en outre des étapes d'impression en sérigraphie supplémentaires permettant de colorer le motif ou l'image imprimé(e).

3. Procédé selon la revendication 2, **caractérisé en ce que** ledit mélange de base comprend des solvants organiques pour les pigments.

4. Procédé selon la revendication 3, **caractérisé en ce que** ledit procédé comprend en outre l'étape consistant à réaliser des lavages supplémentaires de zones non protégées, en utilisant des solvants organiques conçus pour retirer lesdits pigments.

5. Procédé selon la revendication 1, **caractérisé en ce que** ladite pâte ou ledit mélange de base est une pâte ou un mélange d'hydroxyde de sodium et de matériau de charge inerte.

6. Impression par transfert métallisé ou métallisé-pigmenté, **caractérisée en ce que** ladite impression est réalisée par un procédé selon l'une quelconque des revendications précédentes.
